

W. F. NASH.

PROCESS OF RECOVERING SOLVENT FROM COLLOIDED NITROCELLULOSE.  
APPLICATION FILED MAR. 7, 1918.

1,293,515.

Patented Feb. 4, 1919.



INVENTOR

William F. Nash  
BY  
Frank S. Bruser  
ATTORNEY.

WITNESS:

Robt. R. Kitchel.

# UNITED STATES PATENT OFFICE.

WILLIAM F. NASH, OF KENVIL, NEW JERSEY, ASSIGNOR TO HERCULES POWDER COMPANY, OF WILMINGTON, DELAWARE, A CORPORATION OF DELAWARE.

## PROCESS OF RECOVERING SOLVENT FROM COLLOIDAL NITROCELLULOSE.

1,293,515.

Specification of Letters Patent.

Patented Feb. 4, 1919.

Application filed March 7, 1918. Serial No. 220,973.

To all whom it may concern:

Be it known that I, WILLIAM F. NASH, a citizen of the United States, residing at Kenvil, county of Morris, and State of New Jersey, have invented a new and useful Improvement in Processes of Recovering Solvent from Colloidal Nitrocellulose, of which the following is a full, clear, and exact description, reference being had to the accompanying drawings, which form a part of this specification.

In the manufacture of smokeless explosive powder, the final treatment preparatory to drying has for its object the elimination of all the solvent (ether and alcohol) except the small proportion that is to remain in the finished product. This treatment, which involves prolonged distillation and treatment with water, requires four separate operations, a prolonged period of time (about fourteen days), and a considerable amount of labor; and a certain percentage of the solvent is lost. The objects of the present invention are to substantially reduce the time required for solvent extraction, to substantially increase the percentage of solvent recovered, to recover the solvents in condition for immediate use for the purpose for which they were originally used, to reduce the number of operations by preferably effecting the result by means of a single two-step process, and to reduce, or practically eliminate the factor of hand labor and manipulation.

The invention, in its broader aspect, comprises the displacement, from the colloidal guncotton or nitrocellulose, of the ether by alcohol, and the displacement of the alcohol by water, and the recovery of the solvents thus displaced; but the invention also comprises other more specific and subordinate novel features which are hereinafter explained. The invention can be most readily understood from a description of the operation of a simplified apparatus which I have successfully employed to carry out the process on a restricted scale; it, however, being understood that the process is not dependent for its execution upon the employment of any particular apparatus.

The drawing is a diagrammatic view of an apparatus for carrying out the process.

A tank *a* is provided for the reception of the colloidal guncotton, or "green" colloid, which may be in the form of pellets shaped like the finished product, but somewhat larger due to their large solvent content. *b* is a fractionating column connected with tank *a*. *c* is a tank for the reception of alcohol and contains steam coils *d*. *e* is a fractionating column connected with tank *c*. *f* is a tank containing steam coils *g*. A pipe *h* extends to tank *a* and is connected with tanks *c* and *f*, the connections being controlled by valves *i* and *j*. A pump *k* is interposed in pipe *h*. *m* is a return pipe from tank *a* to tank *c*. *n* is a pipe leading from fractionating column *b* to tank *c* and controlled by valve *o*. *p* is a pipe connecting fractionating column *e* with tank *f*. *r* is a valve controlling communication between tank *c* and fractionating column *e*.

At the start of the operation, the colloid in tank *a* is submerged in alcohol of a strength which will be miscible with the ether liberated from the colloid. Tank *c* is charged with alcohol of the same strength as that in tank *a*. By means of pump *k*, an endless circulation is established through tanks *a* and *c* and pipes *h* and *m*. The temperature of the circulating liquor is raised, by means of steam coils *d*, to a temperature between the boiling points of ether and alcohol. A temperature of 55 degrees C. is found to be satisfactory.

The circulating liquor extracts and vaporizes ether and some alcohol. These vapors pass from tanks *a* and *c* into the fractionating column *b*, wherein the alcohol is refluxed and the ether permitted to pass on through condensers and to storage. During this operation the outlet to fractionating column *e* is closed by means of valve *r*.

The operation is continued until the desired proportion of ether contained in the colloid is replaced with alcohol. The valve *i* is now closed, thus cutting off the connection from tank *c* through pipe *h* to tank *a*, and the valve *j* is opened, thus opening communication between tank *f* and tank *a* through pipe *h*. Valve *o* is closed to cut off the pipe connection *n* from tank *c* to fractionating column *b*, and valve *r* is opened to place fractionating column *e* in communica-

2  
 tion with tank *c*. The liquor in tank *c* is heated to boiling and fractionated. The gas condensed in the fractionating column *e* is drawn off through pipe *p* to tank *f*, where it is mixed with water in an amount equaling the volume of alcohol which passes through the fractionating column *e* to the condensers and kept at a temperature of 50-55 degrees C. The liquor flows from tank *f* through pipe *h* into tank *a* and thence through pipe *m* into tank *c*. As the operation proceeds, the content of alcohol in the endless circuit is constantly diminishing until the liquor is almost wholly water.

15 When the material in tank *a* has had enough solvent extracted to give the required residual solvent when dried, the circulation is stopped and the liquor in all three tanks is pumped into tank *e* and the remaining solvent content of the circulating liquor is fractionated off.

The material is now dried in the usual way.

It has been found that the time required for the extraction of the solvent is reduced, by the employment of my process, to about two days. The recovery of the solvent is practically complete and the products recovered are ready for immediate use for the purpose for which they were originally used. The process is a unitary one instead of one involving a number of separate and distinct successive operations. The labor required in the way of manipulation and oversight is reduced to a minimum.

35 Having now fully described my invention, what I claim and desire to protect by Letters Patent is:

1. The process of removing from colloidal nitrocellulose the excess of the ether and alcohol solvent contained therein, which comprises first displacing contained ether by means of alcohol and then displacing contained alcohol by means of water.

45 2. The process of removing from colloidal nitrocellulose that part of the ether and alcohol contained therein which is not to remain in the finished product, which comprises bringing the nitrocellulose in contact with alcohol maintained at a temperature above the boiling point of the ether and below the boiling point of the alcohol until the desired percentage of ether is eliminated by substitution and evaporation, then gradually expelling the alcohol with water until the excess of alcohol is eliminated by substitution, and subsequently drying.

3. The process of removing from colloidal nitrocellulose the excess of alcohol and ether contained therein, which comprises displacing most of the ether with alcohol, and then flowing through the nitrocellulose a current of alcohol while gradually diluting the alcohol with water until the flowing

current is mainly water and until most of the alcohol has been removed by substitution.

4. The process of removing from colloidal nitrocellulose the excess of ether and alcohol contained therein, which comprises flowing a current of alcohol through the nitrocellulose while maintaining the temperature above the boiling point of the ether until the desired percentage of ether is eliminated by substitution and evaporation, and then flowing a current of water through the nitrocellulose and evaporating the alcohol until the excess of alcohol is removed by substitution and evaporation.

5. The process of removing from colloidal nitrocellulose the excess of alcohol and ether contained therein, which comprises displacing most of the ether with alcohol, and then, while maintaining an endless flow of alcohol through the nitrocellulose, gradually adding water to the alcohol while evaporating the alcohol until most of the alcohol has been removed from the nitrocellulose and the flowing current by substitution.

6. The process of removing from colloidal nitrocellulose the excess of ether and alcohol contained therein, which comprises flowing a current of alcohol through the nitrocellulose while maintaining the temperature above the boiling point of the ether until the desired percentage of ether is eliminated by substitution and evaporation, and then, while maintaining the flow of alcohol through the nitrocellulose, gradually evaporating the alcohol and substituting water until most of the alcohol has been removed from the nitrocellulose and until the displacement of the alcohol by water in the flowing current has been practically complete.

7. The process of removing from colloidal nitrocellulose the excess of ether and alcohol contained therein, which comprises flowing a current of alcohol through the nitrocellulose while maintaining the temperature above the boiling point of the ether and fractionally distilling the evaporated ether, and alcohol until the solvent contained in the powder is mainly alcohol, and then with water displacing from the nitrocellulose most of the contained alcohol.

8. The process of removing from colloidal nitrocellulose the excess of the ether-and-alcohol solvent contained therein, which comprises immersing the nitrocellulose in alcohol and flowing the alcohol through the same in an endless circuit while maintaining a temperature above the boiling point of the ether; allowing the evaporated ether and the alcohol carried off therewith to escape from the circuit and separating them by fractionation; then, after the desired displacement from the nitrocellulose of ether with alcohol has been effected, elevating the temperature of the alcohol to effect its gradual evapora-

tion and adding water and continuing the process until the alcohol is substantially eliminated from the circuit and the desired displacement from the nitrocellulose of alcohol with water has been effected, condensing the evaporated alcohol and drying the product, whereby the removal of the solvent is

substantially accelerated and the percentage of recovered solvent substantially increased.

In testimony of which invention, I have 10 hereunto set my hand, at Kenvil, N. J., on this 2nd day of March, 1918.

WILLIAM F. NASH.